

## UNITED STATES PATENT OFFICE

HENRY T. KOENIG, OSCAR A. FISCHER, EARL F. HAFFEY, AND AUDIS B. CLAMPITT, OF DENVER, COLORADO, ASSIGNEES TO R. H. CHANNING, JR., AGENT, OF SAN FRANCISCO, CALIFORNIA

## FLOTATION PROCESS

No Drawing.

Application filed September 21, 1927. Serial No. 221,136.

Our invention relates to reagents for use in the flotation of ores.

In the flotation of many sulfide ores, the flotation of various sulfides selectively from the gangue materials is sought. In some cases a micaceous gangue causes flotation to become involved and costly through the inability to either float it cleanly from the sulfides or depress it to an extent that will prevent its contaminating the various sulfide floats.

It has also been found, in cases, that when conditions are satisfactory for the flotation of mica, or any particular sulfide, the flotation circuit is out of balance, or destroyed for the flotation of other sulfides. In this connection, we have discovered several classes of compounds, or their mixture, which permit not only of regulation of a flotation circuit, but also of better selectivity. The classes of reagents whereby this regulation and selectivity are obtained are: the resins, gums, the gum resins, and the oleo resins. Cited among the above classes of compounds are: Canada balsam, Peru balsam, tolu balsam, benzoin, copal, sandarac, guaiacum, ammoniacum, gamboge; gum dextrin, gum arabic, myrrh, tragacanth, etc.

We have found that some individual gums, etc. work better than others, while some mixtures work better than the individual gums, gum resins or balsams. Our best results thus far have been obtained from gum arabic, myrrh, dextrin, tragacanth, benzoin, and balsam Peru.

For want of a more appropriate term to identify this class of gums, resins, gum resins, oleo resins, adhesives, etc., described herein, the term "gummy adhesive" is used. It is to be understood, however, that this term "gummy adhesive" is used in the special sense hereby indicated, and that any interpretation of the term which is inappropriate to this invention, should not be applied in construing the claims.

Water or alcoholic solutions of the aforesaid compounds, or mixtures thereof, when added with the usual flotation oils and reagents, to a flotation circuit at the stages desired, will permit the operator to control the flotation at these stages. In addition to the selectivity and regulation lent by these compounds, higher grade concentrates can be obtained and better recoveries effected. In order to more clearly show the effectiveness of these reagents, a few examples may be cited:

An ore assaying 1.5% copper; 2.5% zinc; 18% insoluble; 25% iron; 26% sulfur, was ground in a ball mill with lime (1 lb. per ton of ore) and floated for copper, using 0.05 lbs. pine oil per ton of ore and 0.2 lbs. sodium xanthate per ton of ore. After removal of the copper float, 0.75 lbs. copper sulfate, 0.5 lbs. lime, 0.1 lbs. cresylic acid, and 0.1 lbs. sodium xanthate were added and the zinc floated off. This was heretofore the best practice on this ore, and the products obtained assayed as follows:

|                          | Copper   | Zinc     | Insoluble |
|--------------------------|----------|----------|-----------|
|                          | Per cent | Per cent | Per cent  |
| Copper concentrates..... | 10.5     | 5.0      | 21.1      |
| Zinc concentrates.....   | 1.55     | 14.2     | 12.0      |
| Tailings.....            | 0.4      | 0.6      | 14.9      |

The above float was duplicated, adding 1.5 lbs. gum arabic per ton of ore, prior to the copper float, and 0.5 lbs. of gum arabic, and only 0.05 lbs. sodium xanthate per ton of ore, to the zinc float, other conditions being the same.

|                          | Copper   | Zinc     | Insoluble |
|--------------------------|----------|----------|-----------|
|                          | Per cent | Per cent | Per cent  |
| Copper concentrates..... | 13.8     | 2.8      | 2.0       |
| Zinc concentrates.....   | 1.8      | 33.1     | 1.3       |
| Tailings.....            | 0.35     | 0.5      | 15.5      |

By using the same reagents and gum arabic, as above, and increasing the alkalinity, the in-

soluble was floated off leaving most of the sulfides behind for subsequent separation. The analysis of this insoluble (mostly mica) was:

|             | Per cent |
|-------------|----------|
| 5 Insoluble | 85       |
| Iron        | 4.0      |
| Copper      | 0.25     |
| Zinc        | 0.3      |

An attempt to float the insoluble under the same conditions as cited above, but without the use of gum arabic, gave the following float:

|              | Per cent |
|--------------|----------|
| 15 Insoluble | 65       |
| Iron         | 5.6      |
| Copper       | 0.85     |
| Zinc         | 1.2      |

If during a copper or zinc float, iron enters the float in excessive quantities, the addition of gums, gum resins, etc., will completely depress everything tending to float, and the circuit can be readjusted by the addition of the usual flotation oils. By thus "killing" the float, and subsequently adding the usual flotation oils the valuable sulfide sought is floated in preference to the iron. If the insoluble is not floated off before the copper and zinc, it can be depressed by gum arabic and acid, and the iron floated off leaving practically all of the insoluble in the residue. Conditions of alkalinity and acidity together with quantities of the gums, gum resins, resins and oleo resins added govern the flotation of the various sulfide minerals and micaceous insoluble. In cases of "over oiling" or addition of excessive amounts of reagents the circuit can be readjusted and regulated by addition of solutions or mixtures of solutions of various gums, gum resins, oleo resins and balsams, in quantities varying from 0.1 lbs. to 5 lbs. of the dissolved gums, gum resins, oleo resins or balsams, or mixtures thereof, to the ton of ore.

Due to the varying characteristics of ores, it will be appreciated that the particular composition or conditions will vary; but the selection of the composition or conditions can be readily determined by those skilled in the art.

What we claim, is:

- 50 1. In a process of froth flotation of pulp using the known froth flotation reagents, the step of controlling the activity of the froth flotation reagents and controlling the flotation of micaceous matter which consists in adding controlled quantities of a reagent containing a gummy adhesive to the circuit, and subsequently adding further quantities of known froth flotation reagents to the circuit.
- 55 2. In a process of froth flotation of pulp containing miscaceous minerals using known froth flotation reagents, the step of controlling the flotation characteristics of the miscaceous matter which comprises adding to the circuit containing the known flotation

reagents an additional reagent containing a gummy adhesive.

In testimony whereof, we affix our signatures.

HENRY T. KOENIG.  
OSCAR A. FISCHER.  
AUDIS B. CLAMPITT.  
EARL F. HAFFEY.

70

75

80

85

90

95

100

105

110

115

120

125

130